



US007318986B2

(12) **United States Patent**  
**Wu et al.**

(10) **Patent No.:** **US 7,318,986 B2**  
(45) **Date of Patent:** **Jan. 15, 2008**

(54) **PHOTOCONDUCTIVE MEMBERS**

(75) Inventors: **Jin Wu**, Webster, NY (US); **Robert P. Altavela**, Farmington, NY (US); **Linda Ferrarese**, Rochester, NY (US); **Liang-Bih Lin**, Rochester, NY (US)

(73) Assignee: **Xerox Corporation**, Norwalk, CT (US)

(\*) Notice: Subject to any disclaimer, the term of this patent is extended or adjusted under 35 U.S.C. 154(b) by 295 days.

(21) Appl. No.: **11/126,463**

(22) Filed: **May 11, 2005**

(65) **Prior Publication Data**

US 2006/0257769 A1 Nov. 16, 2006

(51) **Int. Cl.**

**G03G 15/02** (2006.01)

(52) **U.S. Cl.** ..... **430/59.6; 430/58.35**

(58) **Field of Classification Search** ..... **430/58.35, 430/58.8, 59.4, 59.6**

See application file for complete search history.

(56) **References Cited**

U.S. PATENT DOCUMENTS

3,121,006 A 2/1964 Middleton et al.  
4,265,990 A 5/1981 Stolka et al.  
4,555,463 A 11/1985 Hor et al.  
4,587,189 A 5/1986 Hor et al.

|                   |         |                             |
|-------------------|---------|-----------------------------|
| 4,921,769 A       | 5/1990  | Yuh et al.                  |
| 5,135,828 A *     | 8/1992  | Yang et al. .... 430/58.75  |
| 5,354,636 A *     | 10/1994 | Ono et al. .... 430/78      |
| 5,473,064 A       | 12/1995 | Mayo et al.                 |
| 5,482,811 A       | 1/1996  | Keoshkerian et al.          |
| 5,874,192 A *     | 2/1999  | Fuller et al. .... 430/59.6 |
| 6,015,645 A       | 1/2000  | Murti et al.                |
| 6,156,468 A       | 12/2000 | Wehlie et al.               |
| 6,177,219 B1      | 1/2001  | Yuh et al.                  |
| 6,255,027 B1      | 7/2001  | Wehlie et al.               |
| 6,287,737 B1      | 9/2001  | Ong et al.                  |
| 6,800,411 B2      | 10/2004 | Tong et al.                 |
| 2004/0013959 A1 * | 1/2004  | Bender et al. .... 430/56   |
| 2004/0161683 A1   | 8/2004  | Wu et al.                   |
| 2004/0161684 A1   | 8/2004  | Wu et al.                   |
| 2005/0014080 A1   | 1/2005  | Tong et al.                 |

OTHER PUBLICATIONS

Diamond, "Handbook of Imaging Materials," Marcel Dekker, Inc, NY, NY. 1991.\*

\* cited by examiner

*Primary Examiner*—Mark F. Huff

*Assistant Examiner*—Peter Vajda

(74) *Attorney, Agent, or Firm*—E. D. Palazzo

(57) **ABSTRACT**

A photoconductive imaging member containing a photogenerating layer, and a charge transport layer containing a binder and a suitable polyimide, and more specifically, an amorphous polyimide.

**27 Claims, No Drawings**

**1**  
**PHOTOCONDUCTIVE MEMBERS**

**CROSS-REFERENCE TO RELATED  
APPLICATIONS**

Illustrated in copending U.S. application Ser. No. 11/126,664, U.S. Publication No. 20060257766 filed concurrently herewith, the disclosure of which is totally incorporated herein by reference, is, for example, a photoconductive imaging member comprised of a photogenerating layer, and a charge transport layer containing a binder and a polyol ester.

Illustrated in U.S. Pat. No. 7,094,509, filed Jul. 18, 2003 and entitled Photoconductive Members, the disclosure of which is totally incorporated herein by reference, is, for example, a photoconductive imaging member comprised of a photogenerating layer, and a charge transport layer containing a binder and a fluoropolymer generated by the free radical polymerization of a fluoroalkyl (methyl) acrylate and an alkyl (methyl) acrylate.

Illustrated in U.S. Pat. No. 6,800,411, the disclosure of which is totally incorporated herein by reference, is, for example, a photoconductive imaging member comprised of a substrate, a photogenerating layer, and a charge transport layer containing a binder and a multi-(methyl) acrylate.

There is illustrated in U.S. Pat. No. 7,037,631, filed Feb. 19, 2003 on Photoconductive Imaging Members, the disclosure of which is totally incorporated herein by reference, a photoconductive imaging member comprised of a supporting substrate, a hole blocking layer thereover, a crosslinked photogenerating layer and a charge transport layer, and wherein the photogenerating layer is comprised of a photogenerating component and a vinyl chloride, allyl glycidyl ether and hydroxy group containing polymer.

There is illustrated in U.S. Pat. No. 6,913,863, filed Feb. 19, 2003 on Photoconductive Imaging Members, the disclosure of which is totally incorporated herein by reference, a photoconductive imaging member comprised of a hole blocking layer, a photogenerating layer, and a charge transport layer, and wherein the hole blocking layer is comprised of a metal oxide; and a mixture of phenolic compounds and a phenolic resin wherein the phenolic compound contains at least two phenol groups.

There is illustrated in U.S. Pat. No. 6,824,940, the disclosure of which is totally incorporated herein by reference, a photoconductive imaging member and thereover an overcoat layer comprised of a polymer with a low dielectric constant and charge transport molecules.

The components, such as photogenerating pigments, charge transport compounds, supporting substrates, hole blocking layers and binder polymers, and processes of the copending applications may be selected for the present disclosure in embodiments thereof.

**RELATED PATENTS**

Illustrated in U.S. Pat. No. 6,015,645, the disclosure of which is totally incorporated herein by reference, is a photoconductive imaging member comprised of a supporting substrate, a hole blocking layer, an optional adhesive layer, a photogenerator layer, and a charge transport layer, and wherein the blocking layer is comprised, for example, of a polyhaloalkylstyrene.

Illustrated in U.S. Pat. No. 6,287,737, the disclosure of which is totally incorporated herein by reference, is a photoconductive imaging member comprised of a supporting substrate, a hole blocking layer thereover, a photoge-

**2**

nerating layer and a charge transport layer, and wherein the hole blocking layer is comprised of a crosslinked polymer derived from the reaction of a silyl-functionalized hydroxy-alkyl polymer of Formula (I) with an organosilane of Formula (II) and water



wherein A, B, D, and F represent the segments of the polymer backbone; E is an electron transporting moiety; X 20 is selected from the group consisting of halide, cyano, alkoxy, acyloxy, and aryloxy; a, b, c, and d are mole fractions of the repeating monomer units such that the sum of a+b+c+d is equal to 1; R is alkyl, substituted alkyl, aryl, or substituted aryl; and R<sup>1</sup>, R<sup>2</sup>, and R<sup>3</sup> are independently selected from the group consisting of alkyl, aryl, alkoxy, aryloxy, acyloxy, halogen, cyano, and amino, subject to the provision that two of R<sup>1</sup>, R<sup>2</sup>, and R<sup>3</sup> are independently selected from the group consisting of alkoxy, aryloxy, acyloxy, and halide.

Illustrated in U.S. Pat. No. 5,473,064, the disclosure of which is totally incorporated herein by reference, is a process for the preparation of hydroxygallium phthalocyanine Type V, essentially free of chlorine, whereby a pigment precursor Type I chlorogallium phthalocyanine is prepared 30 by reaction of gallium chloride in a solvent, such as N-methylpyrrolidone, present in an amount of from about 10 parts to about 100 parts, and preferably about 19 parts with 1,3-diiminoisoindolene (DI<sup>3</sup>) in an amount of from about 1 part to about 10 parts, and preferably about 4 parts DI<sup>3</sup>, for 35 each part of gallium chloride that is reacted; hydrolyzing the pigment precursor chlorogallium phthalocyanine Type I by standard methods, for example acid pasting, whereby the pigment precursor is dissolved in concentrated sulfuric acid and then reprecipitated in a solvent, such as water, or a dilute 40 ammonia solution, for example from about 10 to about 15 percent; and subsequently treating the resulting hydrolyzed pigment hydroxygallium phthalocyanine Type I with a solvent, such as N,N-dimethylformamide, present in an amount of from about 1 volume part to about 50 volume parts, and preferably about 15 volume parts for each weight part of 45 pigment hydroxygallium phthalocyanine that is used by, for example, ballmilling the Type I hydroxygallium phthalocyanine pigment in the presence of spherical glass beads, approximately 1 millimeter to 5 millimeters in diameter, at 50 room temperature, about 25° C., for a period of from about 12 hours to about 1 week, and preferably about 24 hours.

The appropriate components and processes of the above 55 patents may be selected for the present disclosure in embodiments thereof.

**BACKGROUND**

This disclosure is generally directed to imaging members, and more specifically, the present disclosure is directed to multi-layered photoconductive imaging members with a photogenerating layer, a charge transport layer, an optional hole blocking, or undercoat layer (UCL), and wherein the

charge transport layer can be comprised of charge, especially hole transport components and at least one a suitable polyimide, and more specifically an amorphous polyimide. A number of advantages are associated with the members illustrated herein, such as enabling extended life times and excellent wear resistant characteristics; very acceptable compatibility properties with toners generated by emulsion aggregation processes as illustrated in a number of Xerox patents; excellent PIDC cyclic stability at a number of different humidity, for example from about 25 to about 90 percent relative humidity.

In embodiments the imaging members of the present disclosure possess a charge transport or top layer with an excellent resistance to cracking against exposure to chemical vapors emitted from solvents. The charge transport layer's solvent vapor resistance and/or its antiorganic solvent characteristics can be determined by the known solvent vapor induced crystallization test, wherein the imaging member is subjected to exposure by the vapor of common organic solvents, such as for example, methylene chloride, isopropyl alcohol, propylene glycol, a cyclic siloxane of an eight member ring polydimethylsiloxane, tetrahydrofuran, toluene, and the like. As illustrated herein in embodiments, the imaging members of the present disclosure exhibit excellent cyclic/environmental stability; excellent wearability characteristics; enhanced toner image transfer efficiency to the image receiving member; extended lifetimes of, for example, up to 3,500,000 imaging cycles; acceptable and in some instances improved electrical characteristics; members which can be economically prepared with tunable or pre-selected properties depending, for example, on the amount of a suitable polyimide, and more specifically, an amorphous polyimide contained in the charge transport layer; and improved compatibility with a number of toner compositions.

In embodiments, the photogenerating layer can be situated between the charge transport layer and the supporting substrate, and the hole blocking layer in contact with the supporting substrate can be situated between the supporting substrate and the photogenerating layer, which is comprised, for example, of the photogenerating pigments of U.S. Pat. No. 5,482,811, the disclosure of which is totally incorporated herein by reference, especially Type V hydroxygallium phthalocyanine, and generally metal free phthalocyanines, metal phthalocyanines, hydroxy gallium phthalocyanines, perylenes, titanyl phthalocyanines, vanadyl phthalocyanines, selenium, selenium alloys, azo pigments, and the like.

Processes of imaging, especially xerographic imaging and printing, including digital, are also encompassed by the present disclosure. More specifically, the photoconductive imaging members of the present disclosure can be selected for a number of different known imaging and printing processes including, for example, electrophotographic imaging processes, especially xerographic imaging and printing processes wherein charged latent images are rendered visible with toner compositions of an appropriate charge polarity. The imaging members are in embodiments sensitive in the wavelength region of, for example, from about 475 to about 950 nanometers, and in particular from about 650 to about 850 nanometers, thus diode lasers can be selected as the light source. Moreover, the imaging members of this disclosure are useful in color xerographic applications, particularly high-speed color copying and printing processes.

## REFERENCES

Layered photoresponsive imaging members have been illustrated in numerous U.S. patents, such as U.S. Pat. No. 4,265,990, the disclosure of which is totally incorporated herein by reference, wherein there is illustrated an imaging member comprised of a photogenerating layer, and an arylamine hole transport layer. Examples of photogenerating layer components include trigonal selenium, metal phthalocyanines, vanadyl phthalocyanines, and metal free phthalocyanines. Additionally, there is described in U.S. Pat. No. 3,121,006, the disclosure of which is totally incorporated herein by reference, a composite xerographic photoconductive member comprised of finely divided particles of a photoconductive inorganic compound dispersed in an electrically insulating organic resin binder.

Further, in U.S. Pat. No. 4,555,463, the disclosure of which is totally incorporated herein by reference, there is illustrated a layered imaging member with a chloroiridium phthalocyanine photogenerating layer. In U.S. Pat. No. 4,587,189, the disclosure of which is totally incorporated herein by reference, there is illustrated a layered imaging member with, for example, a perylene, pigment photogenerating component. Also known are charge transport aryl amine components, such as N,N'-diphenyl-N,N'-bis(3-methylphenyl)-1,1'-biphenyl-4,4'-diamine dispersed in a polycarbonate binder as a hole transport layer. The above components, such as the photogenerating compounds and the aryl amine charge transport molecules, can be selected for the imaging members of the present disclosure in embodiments thereof.

In U.S. Pat. No. 4,921,769, the disclosure of which is totally incorporated herein by reference, there are illustrated photoconductive imaging members with blocking layers of certain polyurethanes.

Illustrated in U.S. Pat. Nos. 6,255,027; 6,177,219, and 6,156,468, the disclosures of which are totally incorporated herein by reference, are, for example, photoreceptors, and specifically, for example, imaging members containing a hole blocking layer of a plurality of light scattering particles dispersed in a binder, reference for Example I of U.S. Pat. No. 6,156,468, the disclosure of which is totally incorporated herein by reference, wherein there is illustrated a hole blocking layer of titanium dioxide dispersed in a specific linear phenolic binder of VARCUM, available from Oxy-Chem Company.

## SUMMARY

It is a feature of the present disclosure to provide imaging members with many of the advantages illustrated herein, such as extended lifetimes of service of, for example, in excess of about 3,000,000 imaging cycles; excellent electronic characteristics; stable electrical properties; resistance to charge transport layer cracking upon exposure to the vapor of certain solvents; superior surface characteristics; improved wear resistance; compatibility with a number of toner compositions, and the like.

Another feature of the present disclosure relates to the provision of layered photoresponsive imaging members, which are responsive to near infrared radiation of from about 700 to about 900 nanometers.

It is yet another feature of the present disclosure to provide layered photoresponsive imaging members with sensitivity to visible light.

Moreover, another feature of the present disclosure relates to the provision of layered photoresponsive imaging members with mechanically robust and solvent resistant charge transport layers.

In a further feature of the present disclosure there are provided imaging members containing a suitable polyimide, and more specifically, an amorphous polyimide in the top layer of the member, which layer can be, for example, a charge transport layer, a protective overcoating layer, and the like.

Moreover, in yet another feature of the present disclosure there are provided imaging members with optional hole blocking layers comprised of metal oxides, phenolic resins, and optional phenolic compounds, and which phenolic compounds containing at least two, and more specifically two to ten phenol groups or phenolic resins with a weight average molecular weight ranging from about 500 to about 2,000, can interact with and consume aldehyde compounds, such as formaldehyde and other phenolic precursors, thereby chemically modifying the properties for such resins and permitting, for example, a hole blocking layer with excellent efficient electron transport, and which usually results in a desirable lower residual potential  $V_{low}$ .

Aspects of the present disclosure relate to a member comprised of a photogenerating layer, and a charge transport layer containing at least one charge transport component, a suitable polyimide, and more specifically, an amorphous polyimide, and a polymeric binder; a photoconductive imaging member comprised in sequence of a substrate, a photogenerating layer, and a charge transport layer comprised of charge transport molecules, a suitable polyimide, and more specifically, an amorphous polyimide, and a polymeric binder; a photoconductive imaging member comprised of a supporting substrate, a hole blocking layer thereover, a photogenerating layer and a charge transport layer comprised of hole transport molecules, a suitable polyimide, and more specifically, an amorphous polyimide, and a polymeric binder; and optionally a top layer comprised, for example, of known low dielectric components; a photoconductive imaging member wherein the supporting substrate is comprised of a known component, such as a conductive metal substrate; a photoconductive imaging member wherein the conductive substrate is aluminum, aluminized polyethylene terephthalate or a titanized polyethylene naphthalate; a photoconductive imaging member wherein the photogenerating layer is of a thickness of from about 0.05 to about 12 microns; a photoconductive imaging member wherein the charge, such as hole transport layer, is of a thickness of from about 10 to about 75 microns; a photoconductive imaging member wherein the photogenerating layer is comprised of photogenerating pigments dispersed in an optional resinous binder in an amount of from about 5 percent by weight to about 95 percent by weight; a photoconductive imaging member wherein the photogenerating resinous binder is selected from the group consisting of copolymers of vinyl chloride, vinyl acetate and hydroxy and/or acid containing monomers, polyesters, polyvinyl butyral, polycarbonates, polystyrene-b-polyvinyl pyridine, and polyvinyl formals; a photoconductive imaging member wherein the charge transport layer comprises a thermoplastic polymer binder and aryl amine molecules; a photoconductive imaging member wherein the charge transport contains



wherein X is selected from the group consisting of alkyl, alkoxy and halogen, and wherein the aryl amine is dispersed in a resinous binder; a photoconductive imaging member wherein the aryl amine alkyl is methyl, wherein halogen is chloride, and wherein the resinous binder is selected from the group consisting of polycarbonates and polystyrene; a photoconductive imaging member wherein the aryl amine is N,N'-diphenyl-N,N'-bis(3-methyl phenyl)-1,1'-biphenyl-4, 4'-diamine; a photoconductive imaging member wherein the photogenerating layer is comprised of metal phthalocyanines, or metal free phthalocyanines; a photoconductive imaging member wherein the photogenerating layer is comprised of titanyl phthalocyanines, perylenes, alkylhydroxygallium phthalocyanines, hydroxygallium phthalocyanines, or mixtures thereof; a photoconductive imaging member wherein the photogenerating layer is comprised of Type V hydroxygallium phthalocyanine; a method of imaging which comprises generating an electrostatic latent image on the imaging member illustrated herein, developing the latent image, especially wherein developing is accomplished with a toner generated by emulsion/aggregation/coalescence processes; and transferring the developed electrostatic image to a suitable substrate; an imaging member wherein the hole blocking layer phenolic compound is bisphenol S, 4,4'-sulfonyldiphenol; an imaging member wherein the phenolic compound is bisphenol A, 4,4'-isopropylidenediphenol; an imaging member wherein the phenolic compound is bisphenol E, 4,4'-ethylidenebisphenol; an imaging member wherein the phenolic compound is bisphenol F, bis(4-hydroxyphenyl)methane; an imaging member wherein the phenolic compound is bisphenol M, 4,4'-(1,3-phenylenediisopropylidene) bisphenol; an imaging member wherein the phenolic compound is bisphenol P, 4,4'-(1,4-phenylenediisopropylidene) bisphenol; an imaging member wherein the phenolic compound is bisphenol Z, 4,4'-cyclohexylidenebisphenol; an imaging member wherein the phenolic compound is hexafluorobisphenol A, 4,4'-(hexafluoroisopropylidene) diphenol; an imaging member wherein the phenolic compound is resorcinol, 1,3-benzenediol; an imaging member wherein the phenolic compound is hydroxyquinone, 1,4-benzenediol or catechin; an imaging member wherein the phenolic resin is selected from the group consisting of a formaldehyde polymer generated with phenol, p-tert-butylphenol and cresol; a formaldehyde polymer generated with ammonia, cresol and phenol; a formaldehyde polymer generated with 4,4'-(1-methylethylidene) bisphenol; a formaldehyde polymer generated with cresol and phenol; and a formaldehyde polymer generated with phenol and p-tert-butylphenol; an imaging member comprised in the sequence of a supporting substrate, a hole blocking layer, an optional adhesive layer, a photogenerating layer, and a charge transport layer as illustrated herein; an imaging member wherein the adhesive layer is comprised of a polyester with an  $M_w$  of about 45,000 to about 75,000, and an  $M_n$  of from about 30,000 to about 40,000; an imaging member wherein the

photogenerator layer is of a thickness of from about 1 to about 5 microns, and wherein the transport layer is of a thickness of from about 20 to about 75 microns; an imaging member wherein the photogenerating layer is comprised of photogenerating pigments dispersed in a resinous binder in an amount of from about 15 percent by weight to about 90 percent by weight, and optionally wherein the resinous binder is selected from the group comprised of vinyl chloride/vinyl acetate copolymers, polyesters, polyvinyl butyral, polycarbonates, polystyrene-b-polyvinyl pyridine, and polyvinyl formals; and an imaging member wherein the charge transport layer comprises suitable known or future developed components, and more specifically, aryl amines dispersed in a binder polymer and a suitable polyimide, and more specifically, an amorphous polyimide illustrated herein.

The concentration of the polyimide in the photoconductor surface layer, or top layer, such as the charge transport layer, is, for example, from about 0.1 weight percent to 70 weight percent by the weight of total solid contents, and more specifically, from about 3 weight percent to about 40, and yet more specifically, from about 4 to about 7 weight percent based on the weight of total solid contents of the charge transport layer. In embodiments the ratio in weight percentage of a suitable polyimide, and more specifically, an amorphous polyimide, a polymeric binder and the charge transport component of the charge transport layer is from about 70/0/30 to about 1/49/50, and yet more specifically, from about 20/40/40 to about 5/50/55.

An example of a polyimide is, for example, one that is soluble or dispersible in an organic solvent and has high processability and stability. More specifically, a polyimide with, for example, an average molecular weight of 10,000 to 300,000 can be generated heating an acid dianhydride and a diamine in an organic polar solvent in the presence of  $\gamma$ -caprolactone or  $\beta$ -butyrolactone as an acid catalyst.

Also, a useful polyimide may be considered a homopolymer where a single diamine is reacted with a single acid dianhydride, or random or block copolymer thereof when two or more diamines or two or more acid dianhydrides are reacted.

Examples of diamines are aliphatic or alicyclic diamines, and more specifically, two or more compounds in the alternative of the following formulas



15 Examples of acid dianhydrides are aromatic, aliphatic or alicyclic dianhydrides, and more specifically, one or more compounds of the formulas



Organic polar solvents that can be selected include, for example, monochlorobenzene (MCB), tetrahydrofuran (THF), N,N-dimethylformamide (DMF), N,N-dimethylacetamide (DMAc), dimethylsulfoxide (DMSO), N-methyl-2-pyrrolidone (NMP),  $\gamma$ -butyrolactone, and 1,3-dimethyl-2-imidazolidinone.

The polyimide selected can in embodiments be represented by



wherein R<sub>1</sub> is an aromatic hydrocarbon with, for example, about 6 to about 36 carbon atoms like aryl, or an aliphatic or alicyclic hydrocarbon with, for example, from about 1 to about 25 carbon atoms like alkyl; and R<sub>2</sub> is an aliphatic or alicyclic hydrocarbon like alkyl. R<sub>1</sub> can be derived from an acid dianhydride, and R<sub>2</sub> from a diamine.

Specific examples of polyimides selected from the imaging members disclosed herein include P1-100, commercially available from Maruzen Aerican, Inc. Houston, Tex., believed to be of the following formula



wherein n represents the number of segments of, for example, from about 20 to about 1,000, from about 30 to about 100, and more specifically, wherein n is equal to 45.

The thickness of the substrate layer depends on many factors, including economical considerations, electrical characteristics, and the like, thus this layer may be of substantial thickness, for example over 3,000 microns, such as from about 300 to about 500 microns, or of minimum thickness. In embodiments, the thickness of this layer is from about 75 microns to about 300 microns.

The photogenerating layer, which can, for example, be comprised of hydroxygallium phthalocyanine Type V, is in embodiments comprised of, for example, about 60 weight percent of Type V and about 40 weight percent of a resin binder like polyvinylchloride vinylacetate copolymer such as VMCH (Dow Chemical). The photogenerating layer can contain known photogenerating pigments, such as metal phthalocyanines, metal free phthalocyanines, alkylhydroxyl gallium phthalocyanines, hydroxygallium phthalocyanines, perlynes, especially bis(benzimidazo)perlyne, titanyl phthalocyanines, and the like, and more specifically, vanadyl phthalocyanines, Type V hydroxygallium phthalocyanines, and inorganic components such as selenium, selenium alloys, and trigonal selenium. The photogenerating pigment can be dispersed in a resin binder similar to the resin binders selected for the charge transport layer, or alternatively no resin binder need be present. Generally, the thickness of the photogenerator layer depends on a number of factors, including the thicknesses of the other layers and the amount of photogenerator material contained in the photogenerating layers. Accordingly, this layer can be of a thickness of, for example, from about 0.05 micron to about 10 microns, and more specifically, from about 0.25 micron to about 2 microns when, for example, the photogenerator compositions are present in an amount of from about 30 to about 75 percent by volume. The maximum thickness of this layer in embodiments is dependent primarily upon factors, such as

photosensitivity, electrical properties and mechanical considerations. The photogenerating layer binder resin present in various suitable amounts, for example from about 1 to about 50, and more specifically, from about 1 to about 10 weight percent, may be selected from a number of known polymers such as poly(vinyl butyral), poly(vinyl carbazole), polyesters, polycarbonates, poly(vinyl chloride), polyacrylates and methacrylates, copolymers of vinyl chloride and vinyl acetate, phenolic resins, polyurethanes, poly(vinyl alcohol), polyacrylonitrile, polystyrene, and the like. It is desirable to select a coating solvent that does not substantially disturb or adversely affect the other previously coated layers of the device. Examples of coating solvents for the photogenerator layers are ketones, alcohols, aromatic hydrocarbons, halogenated aliphatic hydrocarbons, ethers, amines, amides, esters, and the like. Specific examples are cyclohexanone, acetone, methyl ethyl ketone, methanol, ethanol, butanol, amyl alcohol, toluene, xylene, chlorobenzene, carbon tetrachloride, chloroform, methylene chloride, trichloroethylene, tetrahydrofuran, dioxane, diethyl ether, dimethyl formamide, dimethyl acetamide, butyl acetate, ethyl acetate, methoxyethyl acetate, and the like.

The coating of the photogenerator layer in embodiments of the present disclosure can be accomplished with spray, dip or wire-bar methods such that the final dry thickness of the photogenerator layer is as illustrated herein and can be, for example, from about 0.01 to about 30 microns after being dried at, for example, about 40° C. to about 150° C. for about 15 to about 90 minutes.

Illustrative examples of polymeric binder materials that can be selected for the photogenerator layer are as indicated herein, and include those polymers as disclosed in U.S. Pat. No. 3,121,006, the disclosure of which is totally incorporated herein by reference. In general, the amount of polymer binder that is utilized in the photogenerator layer is from about 0 to about 95 percent by weight, and preferably from about 25 to about 60 percent by weight of the photogenerator layer.

As optional adhesive layers usually in contact with the hole blocking layer and photogenerator layer, there can be selected various known substances inclusive of copolymers, polyamides, poly(vinyl butyral), poly(vinyl alcohol), polyurethane and polyacrylonitrile. This layer is, for example, of a thickness of from about 0.001 micron to about 1 micron. Optionally, this layer may contain effective suitable amounts, for example from 1 to about 10 weight percent, of conductive and nonconductive particles, such as zinc oxide, titanium dioxide, silicon nitride, carbon black, and the like, to provide, for example, in embodiments of the present disclosure further desirable electrical and optical properties.

Aryl amines selected for the charge, especially hole transporting layers, which generally are of a thickness of from about 5 microns to about 75 microns, and more specifically, of a thickness of from about 10 microns to about 40 microns, include molecules of the following formula



wherein X is alkyl, alkoxy, aryl, a halogen, or mixtures thereof, and especially those substituents selected from the group consisting of Cl and CH<sub>3</sub>.

Examples of specific aryl amines are N,N'-diphenyl-N,N'-bis(alkylphenyl)-1,1-biphenyl-4,4'-diamine wherein alkyl is selected from the group consisting of methyl, ethyl, propyl, butyl, hexyl, and the like; and N,N'-diphenyl-N,N'-bis(halophenyl)-1,1'-biphenyl-4,4'-diamine wherein the halo substituent is preferably a chloro substituent. Other known charge transport layer molecules can be selected, reference for example, U.S. Pat. Nos. 4,921,773 and 4,464,450, the disclosures of which are totally incorporated herein by reference.

Examples of the binder materials selected for the charge transport layer include components, such as those described in U.S. Pat. No. 3,121,006, the disclosure of which is totally incorporated herein by reference. Specific examples of polymer binder materials include polycarbonates, polyarylates, acrylate polymers, vinyl polymers, cellulose polymers, polyesters, polysiloxanes, polyamides, polyurethanes, poly(cyclo olefins), and epoxies, and random or alternating copolymers thereof. Preferred electrically inactive binders are comprised of polycarbonate resins with a molecular weight of from about 20,000 to about 100,000 with a molecular weight M<sub>w</sub> of from about 50,000 to about 100,000 being particularly preferred. Generally, the transport layer contains from about 10 to about 75 percent by weight of the charge transport material, and more specifically, from about 35 percent to about 50 percent of this material.

The optional hole blocking or undercoat layers for the imaging members of the present disclosure can contain a number of components including known hole blocking components, such as amino silanes, doped metal oxides, TiSi, a metal oxide like titanium, chromium, zinc, tin and the like, a mixture of phenolic compounds and a phenolic resin or a mixture of 2 phenolic resins, and optionally a dopant such as SiO<sub>2</sub>. The phenolic compounds usually contain at least two phenol groups, such as bisphenol A (4,4'-isopropylidenediphenol), E (4,4'-ethylidenebisphenol), F (bis(4-hydroxyphenyl)methane), M (4,4'-(1,3-phenylenediisopropylidene)bisphenol), P (4,4'-(1,4-phenylene diisopropylidene)bisphenol), S (4,4'-sulfonylidiphenol), and Z (4,4'-cyclohexylidenebisphenol); hexafluorobisphenol A (4,4'-(hexafluoro isopropylidene)diphenol), resorcinol, hydroxyquinone, catechin and the like.

The hole blocking layer can be, for example, comprised of from about 20 weight percent to about 80 weight percent, and more specifically, from about 55 weight percent to about 65 weight percent of a metal oxide, such as TiO<sub>2</sub>, from about 20 weight percent to about 70 weight percent, and more specifically, from about 25 weight percent to about 50 weight percent of a phenolic resin; from about 2 weight percent to about 20 weight percent and, more specifically, from about 5 weight percent to about 15 weight percent of a phenolic compound preferably containing at least two phenolic groups, such as bisphenol S, and from about 2 weight percent to about 15 weight percent, and more specifically, from about 4 weight percent to about 10 weight percent of a plywood suppression dopant, such as SiO<sub>2</sub>. The hole blocking layer coating dispersion can, for example, be prepared as follows. The metal oxide/phenolic resin dispersion is first prepared by ball milling or dynomilling until the median particle size of the metal oxide in the dispersion is less than about 10 nanometers, for example from about 5 to about 9. To the above dispersion, a phenolic compound and dopant are added followed by mixing. The hole blocking layer coating dispersion can be applied by dip coating or web coating, and the layer can be thermally cured after coating. The hole blocking layer resulting is, for example, of

a thickness of from about 0.01 micron to about 30 microns, and more specifically, from about 0.1 micron to about 8 microns. Examples of phenolic resins include formaldehyde polymers with phenol, p-tert-butylphenol, cresol, such as VARCUM™ 29159 and 29101 (OxyChem Company), and DURITE™ 97 (Borden Chemical), formaldehyde polymers with ammonia, cresol and phenol, such as VARCUM™ 29112 (OxyChem Company), formaldehyde polymers with 4,4'-(1-methylethylidene) bisphenol, such as VARCUM™ 29108 and 29116 (OxyChem Company), formaldehyde polymers with cresol and phenol, such as VARCUM™ 29457 (OxyChem Company), DURITE™ SD-423A, SD-422A (Borden Chemical), or formaldehyde polymers with phenol and p-tert-butylphenol, such as DURITE™ ESD 556C (Borden Chemical).

Also included within the scope of the present disclosure are methods of imaging and printing with the photoresponsive devices illustrated herein. These methods generally involve the formation of an electrostatic latent image on the imaging member, followed by developing the image with a toner composition comprised, for example, of thermoplastic resin, colorant, such as pigment, charge additives, and surface additives, reference U.S. Pat. Nos. 4,560,635; 4,298,697 and 4,338,390, the disclosures of which are totally incorporated herein by reference, subsequently transferring the image to a suitable substrate, and permanently affixing the image thereto. In those environments wherein the device is to be used in a printing mode, the imaging method involves the same aforementioned sequence with the exception that the exposure step can be accomplished with a laser device or image bar.

The following Examples are being submitted to illustrate embodiments of the present disclosure. These Examples are intended to be illustrative only and are not intended to limit the scope of the present disclosure. Also, parts and percentages are by weight unless otherwise indicated. Comparative Examples and data are also provided.

#### EXAMPLE I

Four multilayered photoreceptors of the rigid drum design were fabricated by conventional coating technology with an aluminum drum of 34 millimeters in diameter as the substrate. These drum photoreceptors contained the same undercoat layer (UCL) and a charge generating layer (CGL). The only difference was that one photoreceptor, Device I, contained a charge transport layer (CTL) comprising a film forming polymer binder, and a charge transport compound. (Device II) contained the same layers as Device I except that polyimide P1-100, n equal to 45, was incorporated into the charge transport layer. The third device (Device III) contained the same layers as Device I except that polyimide HOP-400 (R<sub>1</sub>=aromatic hydrocarbon, R<sub>2</sub>=aliphatic or alicyclic hydrocarbon, available from Hitachi Cable, Ltd., Ibaraki, Japan) was incorporated into the charge transport layer; and the fourth device contained HOP-500, available from Hitachi Cable, in the charge transport layer.

More specifically, a titanium oxide/phenolic resin dispersion was prepared by ball milling 15 grams of titanium dioxide (STR60NTM, Sakai Company), 20 grams of the phenolic resin (VARCUM™ 29159, OxyChem Company, M<sub>w</sub> of about 3,600, viscosity of about 200 cps) in 7.5 grams of 1-butanol, and 7.5 grams of xylene with 120 grams of 1 millimeter diameter sized ZrO<sub>2</sub> beads for 5 days. Separately, a slurry of SiO<sub>2</sub> and a phenolic resin was prepared by adding 10 grams of SiO<sub>2</sub> (P100, Esprit) and 3 grams of the above phenolic resin into 19.5 grams of 1-butanol and 19.5 grams of xylene. The resulting titanium dioxide dispersion was filtered with a 20 micrometer pore size nylon cloth, and then the filtrate was measured with Horiba Capa 700 Particle Size

13

Analyzer, and there was obtained a median  $\text{TiO}_2$  particle size of 50 nanometers in diameter and a  $\text{TiO}_2$  particle surface area of 30  $\text{m}^2/\text{gram}$  with reference to the above  $\text{TiO}_2$ /VARCUM™ dispersion. Additional solvents of 5 grams of 1-butanol, 5 grams of xylene; and 5.4 grams of the above prepared  $\text{SiO}_2$ NARCUM™ slurry were added to 50 grams of the above resulting titanium dioxide/VARCUM™ dispersion, referred to as the coating dispersion. Then an aluminum drum, cleaned with detergent and rinsed with deionized water, was dip coated with the above generated coating dispersion at a pull rate of 160 millimeters/minute, and subsequently, dried at 145° C. for 45 minutes, which resulted in an undercoat layer (UCL) deposited on the aluminum and comprised of  $\text{TiO}_2$ / $\text{SiO}_2$ NARCUM™ with a weight ratio of about 60/10/40 and a thickness of 4 microns.

A 0.5 micron thick photogenerating layer was subsequently coated on top of the above generated undercoat layer from a dispersion of Type V hydroxygallium phthalocyanine (3 grams) and a vinyl chloride/vinyl acetate copolymer, VMCH ( $M_n=27,000$ , about 86 weight percent of vinyl chloride, about 13 weight percent of vinyl acetate, and about 1 weight percent of maleic acid) available from Dow Chemical (2 grams), in 95 grams of n-butylacetate. Subsequently, a 24  $\mu\text{m}$  thick charge transport layer (CTL) was coated on top of the photogenerating layer from a solution prepared from  $\text{N,N}'$ -diphenyl-N,N'-bis(3-methylphenyl)-1,1'-biphenyl-4,4'-diamine (5 grams) and a film forming polymer binder PCZ-400 [poly(4,4'-dihydroxy-diphenyl-1-1-cyclohexane,  $M_w=40,000$ )] available from Mitsubishi Gas Chemical Company, Ltd. (7.5 grams) dissolved in a solvent mixture of 20 grams of tetrahydrofuran (THF) and 6.7 grams of toluene. The CTL was dried at 120° C. for 40 minutes to provide the photoreceptor Device I.

Devices II, III and IV were as prepared by repeating the above process except that, respectively, P1-100 (n=45), HOP-400 and HOP-500 were contained in the charge transport layer.

The above prepared four photoreceptor devices were tested in a scanner set to obtain photoinduced discharge cycles, sequenced at one charge-erase cycle followed by one charge-expose-erase cycle, wherein the light intensity was incrementally increased with cycling to produce a series of photoinduced discharge characteristic curves from which the photosensitivity and surface potentials at various exposure intensities were measured. Additional electrical characteristics were obtained by a series of charge-erase cycles with incrementing surface potential to generate several voltage versus charge density curves. The scanner was equipped with a scorotron set to a constant voltage charging at various surface potentials. The devices were tested at surface potentials of 500 and 700 volts with the exposure light intensity incrementally increased by means of regulating a series of neutral density filters; the exposure light source was a 780 nanometer light emitting diode. The aluminum drum was rotated at a speed of 55 revolutions per minute to produce a surface speed of 277 millimeters per second or a cycle time of 1.09 seconds. The xerographic simulation was completed in an environmentally controlled light tight chamber at ambient conditions (40 percent relative humidity and 22° C.). Three photoinduced discharge characteristic (PIDC) curves were obtained from the two different pre-exposed surface potentials, and the data was interpolated into PIDC curves at an initial surface potential of 700 volts. These four devices possessed similar electrical performance characteristics. Incorporation of polyimide in charge transport layer did not appear to adversely affect the electrical properties of the imaging members.

14

## EXAMPLE II

Wear resistance tests of the above four devices were performed using a FX469 (Fuji Xerox) wear fixture. The total thickness of each device was measured via Permascope before each wear test was initiated. Then the devices were separately placed into the wear fixture for 50 kcycles. The total thickness was measured again, and the difference in thickness was used to calculate wear rate (nm/kcycle) of the device. The smaller the wear rate the more wear resistant is the imaging member. The wear rate data were summarized as:

| DEVICE | WEAR RATE (nm/kcycle) |
|--------|-----------------------|
| I      | 90 ± 2                |
| II     | 76 ± 1                |
| III    | 76 ± 1                |
| IV     | 70 ± 2                |

Incorporation of polyimide improves wear resistance of the imaging member by about 20 percent.

The claims, as originally presented and as they may be amended, encompass variations, alternatives, modifications, improvements, equivalents, and substantial equivalents of the embodiments and teachings disclosed herein, including those that are presently unforeseen or unappreciated, and that, for example, may arise from applicants/patentees and others.

What is claimed is:

1. A photoconductive imaging member comprised of a photogenerating layer, and a charge transport layer containing a binder, and an amorphous polyimide, and wherein said polyimide is of the formula



wherein n represents the number of segments.

2. An imaging member in accordance with claim 1 comprised of a substrate, a photogenerating layer, and a charge transport layer comprised of a charge transport component, said binder and said polyimide.

3. An imaging member in accordance with claim 2 wherein said polyimide is generated from the reaction of an aliphatic or an alicyclic diamine, and aromatic, aliphatic or alicyclic acid dianhydride.

4. An imaging member in accordance with claim 1 wherein said polyimide possesses a weight average molecular weight of from about 10,000 to about 300,000.

5. An imaging member in accordance with claim 1 wherein said polyimide possesses a weight average molecular weight of from about 10,000 to about 50,000.

6. An imaging member in accordance with claim 1 wherein said polyimide is dispersed or dissolved in said binder, and in said charge transport layer.

7. An imaging member in accordance with claim 1 wherein said polyimide is present in an amount of from about 0.1 to about 70 percent by weight.

8. An imaging member in accordance with claim 1 wherein said polyimide is present in an amount of from about 3 to about 40 percent by weight.

## 15

9. An imaging member in accordance with claim 1 wherein said polyimide is present in an amount of from about 4 to about 7 percent by weight.

10. An imaging member in accordance with claim 1 wherein said polyimide is soluble in said resin binder, and optionally wherein said binder is a polycarbonate.

11. An imaging member in accordance with claim 1 wherein said binder is a polycarbonate, a polyarylate, an acrylate polymer, a vinyl polymer, a cellulose polymer, a polyester, a polysiloxane, a polyamide, a polyurethane, a poly(cyclo olefin), or optionally an epoxy polymer.

12. An imaging member in accordance with claim 1 wherein said polyimide is mixed with said binder, and which binder comprises polycarbonates, polyarylates, acrylate polymers, vinyl polymers, cellulose polymers, polyesters, polysiloxanes, polyamides, polyurethanes, poly(cyclo olefins), and epoxies, and wherein the amount of said polyimide selected is from about 3 to about 7 percent by weight; the amount of said binder is from about 50 to about 5 percent by weight; and the amount of a charge transport component contained in said transport layer is from about 1 to about 50 percent by weight, and wherein the total of said components is about 100 percent.

13. An imaging member in accordance with claim 1 further including a hole blocking layer, and an adhesive layer.

14. An imaging member in accordance with claim 13 wherein said hole blocking layer is comprised of an amino silane, or wherein said hole blocking layer is comprised of a metal oxide, and wherein said layer is in contact with said photogenerating layer and a supporting substrate.

15. An imaging member in accordance with claim 2 wherein said substrate is a rigid drum, or wherein said substrate is a flexible belt.

16. An imaging member in accordance with claim 2 wherein said substrate is comprised of a conductive metal of aluminum, aluminized polyethylene terephthalate, titanized polyethylene terephthalate, or titanized polyethylene naphthalate; said photogenerator layer is of a thickness of from about 0.05 to about 10 microns, and wherein said transport layer is of a thickness of from about 20 to about 70 microns, and wherein said photogenerating layer is comprised of a photogenerating pigment or photogenerating pigments dispersed in a resinous binder, and wherein said pigment or pigments are present in an amount of from about 5 percent by weight to about 95 percent by weight, and wherein the resinous binder is optionally selected from the group comprised of vinyl chloride/vinyl acetate copolymers, polyesters, polyvinyl butyral, polycarbonates, polystyrene-b-polyvinyl pyridine, and polyvinyl formals.

17. An imaging member in accordance with claim 1 wherein the charge transport layer comprises awl amines, and which aryl amines are of the formula



## 16

wherein X is selected from the group consisting of alkyl and halogen.

18. An imaging member in accordance with claim 17 wherein said awl amine is N,N'-diphenyl-N,N-bis(3-methyl phenyl)-1,1'-biphenyl-4,4'-diamine.

19. An imaging member in accordance with claim 1 wherein said photogenerating layer is comprised of metal phthalocyanines, or metal free phthalocyanines.

20. An imaging member in accordance with claim 1 wherein said photogenerating layer is comprised of Type V hydroxygallium phthalocyanine.

21. A method of imaging which comprises generating an electrostatic latent image on the imaging member of claim 1, developing the latent image, and transferring the developed electrostatic image to a suitable substrate.

22. A photoconductive imaging member comprised in sequence of a substrate, a photogenerating layer, and a charge transport layer comprised of charge transport molecules, a binder, and an amorphous polyimide, and wherein said polyimide of the formula



wherein n represents a number of segments.

23. A photoconductor comprised of a substrate, a photogenerating layer, and a charge transport layer comprised of at least one hole transport component, and an amorphous polyimide optionally with a weight average molecular weight from about 10,000 to about 50,000.

24. An imaging member in accordance with claim 1 wherein n is from about 20 to about 1,000.

25. An imaging member in accordance with claim 1 wherein n is 45.

26. An imaging member in accordance with claim 1 wherein n is a member of from about 35 to about 55.

27. A photoconductor comprised in sequence of a substrate, a photogenerating layer, and a charge transport layer comprised of charge transport molecules, a binder, and an amorphous polyimide, and wherein said binder is a polycarbonate and said polyimide is of the formula



wherein n represents a number of from about 20 to about 1,000.